

## UNITED STATES PATENT OFFICE

CLYDE A. BENSON, OF PORTLAND, MAINE, ASSIGNOR TO RAFFOLD PROCESS CORPORATION, OF ANDOVER, MASSACHUSETTS, A CORPORATION OF MASSACHUSETTS

## PAPER MANUFACTURE

No Drawing.

Application filed November 30, 1927. Serial No. 236,885.

In the manufacture of certain grades of paper, such as magazine and book papers, it is the practice to incorporate a loading or filling material into the paper, together with a certain amount of sizing material, in order to produce a product having the desired weight, opacity, printing surface, and water resistance. The loading and sizing materials are incorporated into the paper pulp in the beater engine, and the sizing material precipitated before the pulp is run off into paper on the paper machine. The precipitation of the sizing material is usually effected by an acidic reagent, such as acid salts of the trivalent and divalent metals, alum generally being used where the sizing material employed is rosin size and discoloration of the resulting paper is to be avoided.

Where acidic reagents such as alum have been used to effect the precipitation of sizing material in the presence of loading material, it has heretofore been necessary to employ loading materials which are inert with respect to an acidic reagent, as otherwise reaction is effected upon the loading materials, this not only seriously hindering the sizing operation, but sometimes resulting in reaction products which interfere with the production of good grade paper. For instance, if calcium carbonate is incorporated together with rosin size into paper pulp in the beater engine, and alum added to effect the precipitation of the size, it is found that a selective reaction takes place upon the calcium carbonate, liberating carbon dioxide and producing calcium sulphate, another loading material. To effect a sizing of the pulp in such case, it would be necessary to add sufficient alum not only to precipitate the size, but also to effect the preliminary selective reaction upon the calcium carbonate. But even if sufficient alum were added to effect both these reactions, there would be many serious difficulties in the way of using a loading material such as calcium carbonate. Thus, the beater capacity of a mill would be greatly decreased, for the reaction between calcium carbonate and alum requires considerable time in the presence of fibrous material and size. Moreover, the carbon dioxide liberated during the

reaction produces violent foaming in the beater, and effervescence in the pulp tends to persist even to the paper machine, the bubbles of carbon dioxide being likely to cause imperfections in the finished sheet of paper. Furthermore, the increased expense of alum becomes a factor of considerable importance, particularly where a large amount of calcium carbonate is used.

It might be reasoned, off-hand, that if the size were precipitated on the pulp before incorporating the calcium carbonate, reaction upon the calcium carbonate would be avoided, but research work evidences the fallacy of such reasoning. (See, for example, Sutermeister's Chemistry of Pulp and Paper Making, 1920, page 300.) Thus, after the precipitation of size with alum, an acidic, in fact a distinctly acidic condition, prevails in the pulp. Upon the addition of the desired amount of calcium carbonate to the pulp, reaction immediately takes place upon the calcium carbonate, carbon dioxide being evolved and the precipitated size being degraded or decomposed to such an extent that its sizing effect is practically nullified. Apparently, reaction takes place between the calcium carbonate and both the free acid and precipitated size, the reaction of the calcium carbonate with these materials proceeding in step-by-step fashion or simultaneously. If sufficient calcium carbonate has been added to combine with all the reactable materials, an alkaline condition prevails in the pulp after the reaction has ceased.

In accordance with the present invention, loading materials, such as calcium carbonate, which react with acid reagents are rendered passive to such reagents. This may be accomplished by treating the loading material with emulsified thermoplastic material, such as paraffin, which is substantially inert with respect to both the loading material and the acidic reagent. My invention, may therefore, be applied to great advantage when it is desired to incorporate loading materials, such as calcium carbonate, which react with acidic reagents, into paper pulp to which an acidic reagent is added, for by the use of suitable thermoplastic materials in emulsified condi-

tion, together with the loading material, reaction between the acidic reagent and the loading materials is prevented. The emulsified thermoplastic material further serves as an excellent sizing or waterproofing agent, and hence may be used alone or together with rosin size to render the resulting paper water-resistant. Only a relatively small amount of emulsified thermoplastic material is necessary to prevent reaction between the loading material and acid reagent, for instance 1% and even less of emulsified paraffin (based on dry weight of pulp) preventing reaction between a much larger amount of calcium carbonate and alum. While I am unable to explain precisely how the emulsified paraffin renders the calcium carbonate passive to alum solution, it is my theory that the particles of paraffin which are of colloidal size form a thin film or envelope about the calcium carbonate particles, thus preventing contact of the alum solution with the carbonate particles and avoiding reaction therebetween.

The use of calcium carbonate in the production of sized papers in accordance with the present invention is of considerable commercial importance, as calcium carbonate is produced in large quantities as a waste product in paper mills employing the soda and kraft processes of producing pulp. In these processes, the inorganic content of the spent cooking liquor is smelted to produce a sodium carbonate-containing smelt, which is dissolved to form a smelt solution. The smelt solution is then treated with lime to convert the sodium carbonate into caustic soda, this being accompanied by the precipitation of calcium carbonate or so-called lime sludge, which is separated from the causticized solution to be used for the production of pulp. The calcium carbonate sludge thus obtained is sometimes dumped near the mill, and is often discharged into natural waterways, constituting a nuisance. My invention makes this waste product available for use as a loading material in the manufacture of sized papers, as it requires little expense to condition it for this purpose. It possesses the great advantage over china clay, which is a relatively expensive material customarily used in loading sized papers because of its inert character, in that with a given amount of sizing material it yields a finished paper of much superior water resistance.

The emulsion employed for rendering the calcium carbonate passive to acidic reagents may be prepared from various thermoplastic materials, or mixtures of such materials, e. g., waxes such as paraffin, Montan or carnauba, or even asphalts. Where discoloration of the finished paper is to be avoided. I preferably employ paraffin, together with a small amount of Montan wax, if desired. The paraffin may be emulsified as the internal phase by the use of various emulsifying or dispersing agents,

for instance by the employment of a solution of sodium silicate or by a solution of soap such as rosin size, or by a mixture of both solutions. Inasmuch as results secured indicate that rosin size when used alone and precipitated on the pulp with alum, without the presence of calcium carbonate, gives a better-sized paper than when a corresponding amount of paraffin emulsified in sodium silicate solution is used alone under the same conditions, I preferably employ an emulsion containing both emulsified paraffin and rosin size, the emulsified paraffin rendering the calcium carbonate passive and also serving to size the pulp and the rosin size, at the same time serving to impart its superior sizing effect when precipitated. One emulsion comprising paraffin and rosin size which has been used extensively in the commercial application of my invention is prepared about as follows. Two parts of soda ash is added to 56 parts of water, solution of the soda ash being hastened, if desired, by heating the water. To this solution is added 12 parts of rosin, the mixture being suitably heated and agitated until the saponification reaction between the rosin and soda ash to produce rosin size is complete, this being manifest by almost complete cessation of foaming. To this resulting rosin size, is added 8 parts of paraffin, the paraffin melting in the hot size and becoming emulsified therein as agitation is continued. After thorough agitation of this mixture, 1 part of Montan wax is added during agitation, and the mass is further agitated until the Montan wax has completely melted and emulsified, whereupon the mass is cooled to approximately the melting point of the paraffin and passed through a colloid mill, which ensures substantially complete emulsification of both the paraffin and Montan wax.

The calcium carbonate to be used as a loading material may be incorporated into the emulsion at a suitable stage during its preparation, for instance before it is passed through the colloid mill, or it may be incorporated into the paper pulp in the beater engine independently of the emulsion. If the calcium carbonate is the lime sludge obtained as a waste product from the soda or kraft process of producing pulp, it may be readily conditioned for use as a loading material by removing any dirt or coarse material contained therein, and grinding to ensure a product substantially all of which passes through a 200-mesh sieve. If desired, any free lime present therein may be carbonated, and any sodium salts contained therein removed by washing.

A procedure which may be employed in loading and sizing pulp especially intended for the manufacture of magazine and book papers may be substantially as follows. Six hundred pounds of sulphite pulp (air-dry) and 400 pounds of soda pulp (air-dry) are

added to the beater engine, together with sufficient water to ensure circulation of the mass. Three hundred and seventy-five pounds of finely divided calcium carbonate 5 (bone-dry) is then added in the form of a uniform aqueous paste or sludge, and is thoroughly disseminated throughout the mass of pulp by the operation of the engine. Seventy-eight pounds of emulsion prepared as previously 10 described and containing paraffin and Montan wax emulsified in rosin size solution, is then added to the engine, whereupon the pulp may be beaten to the slowness desired for papermaking. After beating for about, 15 say, 15 minutes, (or longer, if desired), a solution containing 30 pounds of alum is added to effect a precipitation of the rosin size, whereupon beating is continued for awhile and a solution containing 30 pounds 20 of alum is again added to the engine, this ensuring precipitation of substantially all the size and producing a pH value of 7.5 in the pulp, which indicates slight alkalinity. The pulp may then be jordaned, if desired, 25 diluted to papermaking consistency, and run off into any usual paper on a papermaking machine, and calendered, if desired. The resulting dried paper is water-resistant and contains about 27.1% calcium carbonate, and 30 is especially suitable for use as book and magazine paper.

It is to be understood that the foregoing example is illustrative only, and that the various raw materials and proportions therein recited may be varied greatly, depending upon the characteristics of the product which it is desired to produce. Furthermore, a pulp loaded and sized as herein described may be employed in the production of moulded 40 pulp articles which do not require the use of a paper machine.

I am aware of the fact that it has been proposed to use emulsions of various thermoplastic materials, such as paraffin, or asphalt dispersed 45 in water with colloidal clay as a dispersing agent, to size paper pulp in the beater engine, and I do not claim this step per se; but, so far as I am aware, I am the first to render inert or inactive a loading material, 50 such as calcium carbonate or waste lime sludge, capable of reacting with a precipitating agent such as alum, by the employment of an inert thermoplastic, and thus to secure the benefits and advantages which I have hereinbefore pointed out.

Having thus described certain embodiments of my invention, it is evident that change and modification might be made therein without departing from the spirit or scope 60 of invention as defined in the appended claims.

What I claim is:

1. A method of rendering finely divided calcium carbonate passive to the action of 65 alum solution, which comprises treating such

carbonate with paraffin emulsified in an aqueous solution of rosin size.

2. A method of loading and sizing paper, which comprises incorporating into paper pulp finely divided calcium carbonate together with a paraffin-rosin size emulsion, 70 adding an acidic reagent to precipitate the size, and running the pulp off on a paper machine.

3. A method of loading and sizing paper, 75 which comprises incorporating into paper pulp finely divided calcium carbonate together with a paraffin-rosin size emulsion, adding alum to precipitate the size, and running the pulp off on a paper machine.

4. A method of loading and sizing paper, 80 which comprises incorporating into paper pulp finely divided calcium carbonate together with a rosin size emulsion of paraffin and Montan wax, adding alum to ensure precipitation of the size but without producing an acidic condition in the pulp, and running the pulp off on a paper machine.

5. A loaded and well-sized paper containing 85 calcium carbonate, rosin size, and a thermoplastic material inert with respect to said calcium carbonate.

6. A loaded and well-sized paper containing calcium carbonate, rosin size, and paraffin.

7. A method of sizing and loading paper pulp involving the use of acidic precipitating 90 agents and loading materials which react with such agents, which comprises incorporating such loading materials into the pulp together with a rosin size emulsion of thermoplastic material which renders the loading materials passive to such agents, and then adding such agents to effect a precipitation 95 of the size and thermoplastic material on the fibers.

In testimony whereof I have affixed my signature. 105

CLYDE A. BENSON.

110

115

120

125

130